



US007672626B2

(12) **United States Patent**  
**Uchino et al.**

(10) **Patent No.:** **US 7,672,626 B2**  
(45) **Date of Patent:** **Mar. 2, 2010**

(54) **DEVELOPING ROLLER AND IMAGE FORMING METHOD EMPLOYING THE SAME**

(75) Inventors: **Satoshi Uchino**, Tokyo (JP); **Nobuaki Kobayashi**, Tokyo (JP); **Takeo Oshima**, Tokyo (JP); **Okushi Okuyama**, Tokyo (JP); **Kouichi Sugama**, Tokyo (JP)

(73) Assignee: **Konica Minolta Business Technologies, Inc.**, Tokyo (JP)

(\*) Notice: Subject to any disclaimer, the term of this patent is extended or adjusted under 35 U.S.C. 154(b) by 565 days.

(21) Appl. No.: **11/678,314**

(22) Filed: **Feb. 23, 2007**

(65) **Prior Publication Data**

US 2007/0269239 A1 Nov. 22, 2007

(30) **Foreign Application Priority Data**

May 18, 2006 (JP) ..... 2006-138692

(51) **Int. Cl.**  
**G03G 15/08** (2006.01)

(52) **U.S. Cl.** ..... 399/286; 399/279

(58) **Field of Classification Search** ..... 399/279,  
399/286

See application file for complete search history.

(56)

**References Cited**

**U.S. PATENT DOCUMENTS**

2004/0248025 A1 \* 12/2004 Miyakawa ..... 430/107.1  
2007/0269240 A1 \* 11/2007 Uchino et al. ..... 399/286

\* cited by examiner

*Primary Examiner*—David M Gray

*Assistant Examiner*—Ryan D Walsh

(74) *Attorney, Agent, or Firm*—Lucas & Mercanti, LLP

(57)

**ABSTRACT**

An objective is to provide a developing roller in which increase of residual potential is inhibited during repetitive operation without deteriorating interlayer adhesion, and prepared is a layer immediately below the surface capable of preventing fog caused by toner scattering, accompanied with a surface layer capable of preventing stains formed from foreign matters adhered to the surface, as well as preventing image unevenness since toner electrification is even under the presence of appropriate elasticity, and also to provide a image forming method employing the developing roller. Disclosed is a developing roller possessing an elastic layer made of silicone rubber provided around a conductive shaft, and a plurality of resin layers further provided on the elastic layer, wherein an outermost surface layer among the resin layers comprises silicone copolymerization polyurethane; and a layer immediately below the surface layer comprises a polyurethane resin-silica hybrid.

**6 Claims, 3 Drawing Sheets**



FIG. 1



FIG. 2



FIG. 3 ( a )



FIG. 3 ( b )



FIG. 4



FIG. 5



## 1

**DEVELOPING ROLLER AND IMAGE  
FORMING METHOD EMPLOYING THE  
SAME**

This application claims priority from Japanese Patent Application NO. 2006-138692 filed on May 18, 2006, which is incorporated herein by reference.

**FIELD**

The present invention relates to a developing roller installed in an image forming apparatus employing an electrophotographic process used for a printer, a facsimile receiver and so forth, and specifically to a developing roller used for a developing device employing a non-magnetic single component development process and an image forming method utilizing the developing roller.

**BACKGROUND**

Currently, a widely available electrophotographic image forming method is a method in which a final image is formed via a fixing process after transferring into a plain paper sheet a toner image on an electrostatic latent image carrier, which is formed via a developing process to visualize an electrostatic latent image with toner, by bringing a charge-provided toner into contact with the electrostatic latent image formed on the electrostatic latent image carrier (usually referred to as an electrophotographic photoreceptor), or by making the toner to face the electrostatic latent image carrier via a narrow spacing.

As development processes to form toner images, there are a double component development process in which toner is charged and developed employing a double component developer composed of a carrier and the toner, and also a single component development process in which a developer consisting of toner is conveyed by a developing roller, and charged via friction with a developer regulating member or such to conduct a development treatment. This single component development process has widely been used in recent years since no carrier needs to be used in this process, and a developing device can also be simplified. With the recent development of colorization, attention has been focused on a non-magnetic single component process employing toner with no content of a magnetic material since the colorization is possible with it.

This process differing from the double component development process has the advantage that the development device mechanism is not complicated, and is easily downsized, since friction of only toner is caused with an electrification member without using a carrier, or electrification is caused by pressing the carrier on the developing roller surface. As the result, it is further a feature that this process is also usable for a color image forming apparatus usually employing at least 4 development mechanisms.

Usually, a developing roller comprising an elastic layer composed of silicone rubber provided around the outer circumferential surface of a conductive shaft, for example, has been utilized for a developing roller with this non-magnetic single component development process. A developing device having a very simple mechanism is to be employed since a toner thin layer is formed on the developing roller using an electrification member such as a metal plate or a roller, and friction is caused with this, in order to charge the toner.

This developing roller comprises an elastic layer composed of a rubber elastic body such as silicone rubber provided around the outer circumferential surface of a shaft (or a

## 2

spindle) made of a metal or a conductive resin, but a surface layer composed of a fluorine-containing rubber is formed on the elastic layer in order to provide electrification to toner or to provide toner conveyance. It is commonly known that the fluorine-containing rubber is employed to prevent toner adhesion and fusing to this surface layer. In order to form a fluorine-containing rubber layer on the elastic layer, it is also known that an intermediate layer composed of a silane coupling agent is formed on the elastic layer surface, and a coated layer composed of a fluorine-containing rubber as a principal component is further formed on the intermediate layer (refer to Patent Document 1).

The non-magnetic single component development is capable of receiving and transferring electric charge between the toner and the developing roller, and counter electric charge of the toner is built up on the developing roller surface. This counter electric charge is removed by leaking it into the developing roller to constantly neutralize charge on the developing roller surface. However, when the foregoing structure is employed, no charge formed on a surface layer is effectively leaked since an intermediate layer serves as a barrier layer in this case, whereby residual charge on the developing roller surface is increased, resulting in occurrence of a problem such as scattering of toner and so forth.

(Patent Document 1) Japanese Patent O.P.I. Publication 8-190263

**SUMMARY**

As described above, in a conventional roller, increase of residual potential is generated during repetitive operation under the influence of an insulating silane coupling agent layer (intermediate layer). As a result, there has been a problem such that scattered toner and so forth are generated. The present invention was made to solve this problem.

That is, it is an object of the present invention to provide a developing roller in which increase of residual potential is inhibited during repetitive operation without deteriorating interlayer adhesion, and prepared is a layer immediately below the surface capable of preventing fog caused by toner scattering, accompanied with a surface layer capable of preventing stains formed from foreign matters adhered to the surface, as well as preventing image unevenness since toner electrification is even under the presence of appropriate elasticity, and also to provide a image forming method employing the developing roller. Disclosed is a developing roller comprising an elastic layer made of silicone rubber provided around a conductive shaft, and a plurality of resin layers further provided on the elastic layer, wherein an outermost surface layer among the resin layers comprises silicone copolymerization polyurethane as a principal component, and a layer immediately below the surface layer comprises a polyurethane resin-silica hybrid as a principal component.

**BRIEF DESCRIPTION OF THE DRAWINGS**

Embodiments will now be described, by way of example only, with reference to the accompanying drawings which are meant to be exemplary, not limiting, and wherein like elements numbered alike in several figures, in which:

FIG. 1 is a schematic cross-sectional view showing an example of the developing roller of the present invention;

FIG. 2 is a schematic configuration diagram of a die used for a method of manufacturing a base roller of the present invention;

FIG. 3(a) is a side view of the developing roller;

FIG. 3(b) is a schematic diagram to explain a measuring method of interlayer adhesion between resin layers of the developing roller;

FIG. 4 is a schematic cross-sectional illustration of a developing device employed in an image forming method of the present invention; and

FIG. 5 is a schematic configuration diagram to explain a measuring method of volume resistivity of the developing roller.

### DESCRIPTION OF THE PREFERRED EMBODIMENTS

In order to solve the above-described problems, disclosed is a developing roller comprising an elastic layer made of silicone rubber provided around a conductive shaft (spindle), and a plurality of resin layers further provided on the elastic layer, wherein an outermost surface layer among the resin layers comprises silicone copolymerization polyurethane as a principal component, and a layer immediately below the surface layer comprises a polyurethane resin-silica hybrid as a principal component.

That is, after considerable effort, intensive studies concerning a coated layer-forming material have been made by the inventors in order to obtain a developing roller in which no increase of residual potential is generated during repetitive operation. As the result, it was found out that sufficient charge leakage, accompanied with excellent adhesiveness was accomplished, whereby increase of residual potential was inhibited during repetitive operation by forming an adhesive layer as a resin layer comprising a polyurethane resin-silica hybrid as a principal component and a surface layer as a resin layer comprising silicone copolymerization polyurethane as a principal component.

(Structure 1) A developing roller comprising an elastic layer made of silicone rubber provided around a conductive shaft, and a plurality of resin layers further provided on the elastic layer, wherein an outermost surface layer among the resin layers comprises silicone copolymerization polyurethane as a principal component, and a layer immediately below the surface layer comprises a polyurethane resin-silica hybrid as a principal component.

(Structure 2) The developing roller of Structure 1, wherein a silane moiety content in the polyurethane resin-silica hybrid is 1.0-30.0% by weight.

(Structure 3) The developing roller of Structure 1 or 2, wherein the polyurethane resin-silica hybrid comprises a urea bond.

(Structure 4) An image forming method comprising the steps of conveying a developer comprising a toner to a developing region with a developing roller, and developing an electrostatic latent image formed on an electrostatic latent image carrier for visualization, wherein the developing roller comprises an elastic layer made of silicone rubber provided around a conductive shaft, and a plurality of resin layers further provided on the elastic layer, and wherein an outermost surface layer among the resin layers comprises silicone copolymerization polyurethane as a principal component, and a layer immediately below the surface layer comprises a polyurethane resin-silica hybrid as a principal component.

(Structure 5) The image forming method of Structure 4, wherein a silane moiety content in the polyurethane resin-silica hybrid is 1.0-30.0% by weight.

(Structure 6) The image forming method of Structure 4 or 5, wherein the polyurethane resin-silica hybrid comprises a urea bond.

Incidentally, in the present invention, containing a compound as a principal component means the compound having a content of at least 50% by weight, and a silane moiety means a moiety having a silane or siloxane structure. In addition, in the present invention, an outermost surface layer immediately above a resin layer or resin layers means a surface layer. Further, a layer immediately below a surface layer means a layer under a surface layer, which is adjacently brought into contact with the surface layer.

It was found out in the present invention that an insulating adhesive layer was not merely formed above an elastic layer made of silicone rubber, but a silicone based resin layer formed as a surface layer was formed immediately above an adhesive layer composed of a so-called hybrid resin structure to solve the problem. A layer having a high affinity for the surface layer and the elastic layer, which serves as an adhesion layer, is used to improve adhesiveness, and further to improve closely attached contact. On the other hand, it is assumed that the buildup of electric charges is generated when the adhesive layer itself has become an insulated layer. Therefore, after considerable effort during intensive studies, the inventors have found out that the buildup of electric charges can be prevented by employing the foregoing hybrid contained in the adhesion layer.

Silicone copolymerization polyurethane may be used for a surface layer in view of toner conveyance and charging of toner, and further in order to prevent toner adhesion and fusing. It is for this reason that the toner adhesion and fusing can be prevented since a low surface energy state is possible to be produced by using the silicone component. However, a resin consisting of this silicone component can not improve adhesion to other layers such as an elastic layer and so forth, and layer characteristics are to be deteriorated. Further, charge-providing capability to toner can not be increased. Therefore, a component having a polar group is preferably usable in combination. However, when each of two components is used singly, and employed for an admixture, it is difficult to evenly disperse components having a different level of polarity, though a resin component having a polarity and a silicone resin component having a low level of polarity are desired to be contained via even dispersion. After considerable effort during intensive studies, the inventors have also found out that use of a silicone copolymerization urethane resin including both characteristics in one resin is substantially effective. Since this polymerization resin contains a silicone component and an urethane component in the molecule, the urethane component contributes to adhesion to other layers on the one hand, and the silicone component functions to produce the surface at a low surface energy state, on the other. Further, since both components coexist in a molecule, the above-described even dispersion becomes excellent.

On the other hand, as an adhesive layer, a silane coupling agent is not merely used, but a polyurethane resin-silica hybrid is employed. This structure is described later, but it has a polyurethane unit contained in a moiety, and has a high affinity with silicone copolymerization polyurethane constituting a surface layer, whereby adhesiveness can be improved. Further, since not only adhesion to silicone rubber constituting an elastic layer is improved by possessing the silica hybrid structure, but also the existence of a silica unit inorganic structure simultaneously makes capable of acting as an electric charge leakage point, it is assumed that the electric charges built up on the developing roller surface can be prevented, whereby problems of the present invention have been solved.

While the preferred embodiments of the present invention have been described using specific terms, such description is for illustrative purposes only, and it is to be understood that changes and variations may be made without departing from the spirit or scope of the appended claims.

#### DETAILED DESCRIPTION OF THE INVENTION

Next, the embodiments of the present invention will be explained in detail.

##### [Developing Roller]

A conductive shaft is employed as a spindle for a developing roller, and a conductive elastic layer made of silicone rubber, an intermediate layer composed of a polyurethane resin-silica hybrid as a principal component and a surface layer composed of a silicone copolymerization polyurethane resin as a principal component are formed around the shaft.

FIG. 1 shows a schematic cross-sectional view of developing roller 1 of the present invention. Developing roller 1 is composed of conductive shaft (spindle) 2, elastic layer 3, intermediate layer 4 and surface layer 5.

##### (Conductive Shaft)

The conductive shaft constituting a spindle is preferably made of conductive metal since the shaft serves as a member by which electric charge built up on the developing roller surface is leaked. Typical examples thereof include conductive metals such as stainless steel (SUS304, for example) having a diameter of 1.0-30 mm, iron, aluminum, nickel, an aluminum alloy and a nickel alloy. Further, the shaft may also be composed of conductive resin.

##### (Elastic Layer)

Silicone rubber employed for an elastic layer of the present invention which may be silicone rubber conventionally used in this industry is prepared by adding an inorganic filler, benzoyl peroxide and so forth into organopolysiloxane, and subsequently vulcanizing and curing the resulting after conducting kneading and molding processes. It, for example, can be obtained by crosslinking methylvinylpolysiloxane made of dimethylpolysiloxane and methylvinylsiloxane with organic peroxide. Though the elastic modulus depends on the degree of crosslinking, an elastic body having a JIS A hardness of approximately 10-60° is preferably employed in the present invention.

This elastic layer having low resistivity obtained by adjusting resistivity is also employed. In order to make resistivity lower, low resistive components such as carbon black, graphite, zinc oxide, tin oxide and titanium oxide are preferably contained. In this case, the usable material preferably has a volume resistivity of  $1 \times 10^{-4}$ - $1 \times 10^4 \Omega \cdot \text{cm}$ . Particularly preferable are graphite, Ketjen black and acetylene black. Further, the addition amount is not specifically limited, but the addition amount is preferably 10-100 parts, based on 100 parts of silicone rubber.

##### {Resin Layer (Intermediate Layer)}

A layer immediately below the surface layer of the present invention comprises a layer composed of a polyurethane resin-silica hybrid as a principal component. This has a polyurethane moiety, and is united with a silica structure. Further, this is not particularly limited, but it, for example, can be prepared by a method described in Japanese Patent O.P.I. Publication No. 2002-220431. That is, it is produced with polyhydric alcohol and a polyisocyanate compound, and the polyurethane resin-silica hybrid can be prepared by curing an alkoxy group-containing silane modified polyurethane resin obtained via reaction of (1) a polyurethane resin having a

functional group reactive to an epoxy group and (2) an epoxy group-containing alkoxy silane partial condensate acquired via dealcoholization reaction of (A) an epoxy compound having at least a hydroxyl group in a molecule and (B) an alkoxy silane partial condensate. In addition, a urea bond may also be formed by reacting an isocyanate group and an amine group via addition of amine during reaction. It is preferable that intermolecular adhesion is improved by coexisting a urea bond and an urethane bond, whereby durability is also improved.

The polyhydric alcohol is not particularly limited, but preferably provided are polyester polyol, polycarbonate polyol, polyether polyol and polyolefin polyol which have a hydroxyl group at the terminal. The polyhydric alcohol having a certain level of high molecular weight is preferable in view of improving elasticity, together with mechanical properties of a hardened material, and is preferably a number average molecular weight of 1000-6000. In addition, the number average molecular weight can be determined as a styrene conversion number average molecular weight employing a GPC (gel permeation chromatography). Of the above-described polymer polyols, polyester polyol and polycarbonate polyol are specifically preferable in view of various properties such as high temperature durability of the resulting polyurethane resin-silica hybrid and so forth.

Examples of the polyester polyol include commonly known, various saturated or unsaturated low molecular glycols such as ethylene glycol, diethylene glycol, triethylene glycol, 1,2-propanediol, 1,3-propanediol, 1,3-butanediol, 1,4-butanediol, neopentyl glycol, pentanediol, 3-methyl-1,5-pentanediol, 1,6-hexanediol, octanediol, 1,4-butyne diol, dipropylene glycol; alkylglycidyl ethers such as n-butylglycidyl ether and 2-ethylhexylglycidyl ether; monocarboxylic acid glycidyl esters such as versatic acid glycidyl ester and so forth; dibasic acid or acid anhydride thereof, and dimer acid such as adipic acid, maleic acid, fumaric acid, acid phthalic anhydride, isophthalic acid, terephthalic acid, succinic acid, axalic acid, malonic acid, glutaric acid, pimelic acid, azelaic acid, sebatic acid and suberic acid; and polyester polyols obtained via dehydration-condensation of castor oil and its fatty acid or via ring-opening polymerization of a cyclic ester compound.

Polycarbonate polyols can be prepared via commonly known reaction such as demethanol condensation reaction of polyhydric alcohol and dimethylcarbonate, deurethane condensation reaction of polyhydric alcohol and diphenyl carbonate, or deethyleneglycol condensation reaction of polyhydric alcohol and ethylene carbonate. Examples of the polyhydric alcohol employed in this reaction include commonly known various saturated or unsaturated low molecular glycols such as 1,6-hexanediol, diethylene glycol, Propylene glycol, 1,3-butanediol, 1,4-butanediol, neopentylglycol, pentane diol, 3-methyl-1,5-pentanediol, octanediol, 1,4-butyne diol and dipropylene glycol; and alicyclic glycols such as 1,4-cyclohexane diglycol and 1,4-cyclohexane dimethanol.

Examples of polyester polyols include polyethylene glycol, polypropylene glycol and polyoxytetramethylene glycol prepared via ring-opening polymerization of ethylene oxide, propylene oxide or tetrahydrofuran.

Commonly known various aromatic, fatty or alicyclic polyisocyanates are usable as a polyisocyanate compound being a composition component in polyurethane resin (1), and a diisocyanate compound is preferable in view of providing elasticity.

Examples thereof include 1,5-naphthylene diisocyanate, 4,4'-diphenylmethane diisocyanate, 4,4'-diphenylmethane diisocyanate, 4,4'-dibenzylisocyanate, dialkyl-

diphenylmethane diisocyanate, tetraalkyldiphenylmethane diisocyanate, 1,3-phenylene diisocyanate, 1,4-phenylene diisocyanate, tolylene diisocyanate, butane-1,4-diisocyanate, hexamethylene diisocyanate, isopropylene diisocyanate, methylene diisocyanate, 2,2,4-trimethylhexamethylene diisocyanate, 2,4,4-trimethylhexamethylene diisocyanate, cyclohexane 1,4-diisocyanate, xylylene diisocyanate, hydrogenated xylylene diisocyanate, isophorone diisocyanate, lysine diisocyanate, dicyclohexylmethane-4,4'-diisocyanate, 1,3-bis(isocyanatemethyl)cyclohexane, methylcyclohexane diisocyanate, m-tetramethylxylylene diisocyanate, and dimer diisocyanate in which a carboxyl group in a dimer acid is transformed into isocyanate group.

A chain extension agent for extending a molecular chain is also usable for polyurethane resin (1). Examples of the chain extension agent include low molecular glycols described in the foregoing paragraph of polyester polyol, for example; glycols having a carboxyl group in a molecule such as dimethylolpropionic acid or dimethylolbutanoic acid; polyamines such as dimerdiamine and so forth in which a carboxyl group in ethylenediamine, propylenediamine, hexamethylenediamine, triethylenetetramine, diethylenetriamine, isophoronediamine, dicyclohexylmethane-4,4'-diamine or a dimer acid is transformed into an amino group; and polyamines having a carboxyl group in a molecule such as L-lysine or L-arginine. A urea bond can be formed by providing amines as the chain extension agent. That is, the amount of this urea bond is preferably 1-10 mol %, based on the urethane bond. The amount can be adjusted by adding 1-10 mol % after glycols are to be set to 90-99 mol % during reaction. The interaction through an intermolecular hydrogen bond is generated via coexistence of the urea bond and the urethane bond in a molecule, whereby durability and adhesion of the resulting resin layer can be improved. In the case of the amount of the urea bond being too small, no adhesion can be improved since this intermolecular interaction is deteriorated. On the other hand, in the case of the amount of the urea bond being excessive, adhesion is further lowered since repulsion in the excessive amount of urea bond is produced through the intermolecular interaction is more or less observed.

A polymerization terminator for adjusting a molecular weight is also usable for the polyurethane resin of the present invention. Examples of the polymerization terminator include alkylmonoamines such as di-n-butylamine or n-butylamine; monoamines having a carboxyl group in a molecule such as D-alanine or a D-glutamic acid; alcohols such as ethanol, isopropyl alcohol and so forth; and alcohols having a carboxyl group in a molecule such as a glycolic acid and so forth.

A functional group having an epoxy group in polyurethane resin (1) together with reactivity may be at the terminal or in the principal chain of polyurethane resin (1). Examples of the functional group include a carboxyl group, a sulfonate group, a phosphate group, an acidic group, an amino group, a hydroxyl group, a mercapto group and so forth. Of these, an acidic group and an amino group are preferable in view of reactivity with an epoxy group and functional group providing easiness. A method of providing an acidic group in polyurethane resin (1) is not limited, but a functional group can be provided by using a compound containing the foregoing functional group as the aforementioned chain extension agent or polymerization terminator.

As the method of producing polyurethane resin (1) employed in the present invention, provided are a one step method in which polymeric polyol, a diisocyanate compound, and at least one of the chain extension agent and

polymerization terminator if desired are simultaneously reacted in an appropriate solvent; and a two step method in which polymeric polyol and a diisocyanate compound are reacted under the condition of an excessive amount of isocyanate group to prepare a prepolymer having an isocyanate group at the polymeric polyol terminal, and subsequently reacted with at least one of the chain extension agent and polymerization terminator in an appropriate solvent. The two step method is preferable in order to obtain a homogeneous polymer solution. Examples of commonly known solutions usable in these methods include aromatic solutions such as benzene, toluene, xylene and so forth; ester based solutions such as ethyl acetate, butyl acetate and so forth; alcohol based solutions such as methanol, ethanol, isopropanol, n-butanol, diacetone alcohol and so forth; ketone based solutions such as acetone, methylethyl ketone, methylisobutyl ketone and so forth; and other solutions such as dimethylformamide, dimethylacetamide, ethylene glycoldimethyl ether, tetrahydrofuran, cyclohexanone and so forth. These can be used singly or in mixture of at least two kinds.

Further, a method of incorporating an amino group into polyurethane resin (1) is not limited, but polyamines may be reacted so as to make the amount of the amino group to be excessive with respect to the isocyanate group of the prepolymer at the terminal. The amount of an epoxy group-reactive functional group in polyurethane resin (1) is not specifically limited, but 0.1-20 KOHmg/g is commonly preferable. In the case of an amount of less than 0.1 KOHmg/g, plasticity and heat resistance of a polyurethane resin-silica hybrid are degraded. On the other hand, in the case of an amount exceeding 20 KOHmg/g, moisture resistance of the polyurethane resin-silica hybrid tends to be deteriorated. In addition, one having a urea bond in a polyurethane resin is further preferable in view of interlayer adhesion.

Epoxy group-containing alkoxy silane partial condensate (2) is prepared via dealcoholization reaction of epoxy compound (A) with alkoxy silane partial condensate (B).

As for epoxy compound (A), the number of epoxy group is not limited, provided that an epoxy compound contains one hydroxyl group in a molecule. Epoxy compound (A) having at most 15 carbon atoms is also preferable, since the low molecular weight epoxy compound exhibits good compatibility together with a high heat resistance property and adhesion-providing effect with respect to alkoxy silane partial condensate (B). Specific examples thereof include monoglycidyl ethers having one hydroxyl group at a molecular terminal obtained via reaction of water, dihydric alcohol or phenols with epichlorohydrin; polyglycidyl ethers having one hydroxyl group at a molecular terminal obtained via reaction of polyhydric alcohol like trihydric alcohol or higher hydric such as glycerin, pentaerythritol or such with epichlorohydrin; epoxy compounds having one hydroxyl group at a molecular terminal obtained via reaction of aminomonoalcohol with epichlorohydrin; and alicyclic hydrocarbon monooxides (epoxidized tetrahydrobenzyl alcohol) having one hydroxyl group at a molecular terminal. Of these epoxy compounds, glycidol is excellent in view of heat resistance-providing effect, and is also most preferable since high reactivity is produced with alkoxy silane partial condensate (B).

A hydrolysable alkoxy silane monomer represented by following Formula (a) is hydrolyzed in the presence of an acidic or alkaline water, and condensed partially to obtain usable alkoxy silane partial condensate (B).



Formula (a)

wherein p is 0 or 1; R<sup>1</sup> represents a lower alkyl group, an aryl group or an unsaturated fatty group which may have a

functional group combined directly with a carbon atom; R<sup>2</sup> represents a methyl group or an ethyl group; and R<sup>2</sup>'s each may be the same or be different.

Examples of the hydrolyzable alkoxy silane monomer include tetraalkoxy silanes such as tetramethoxy silane, tetraethoxy silane, tetrapropoxysilane, tetraisopropoxysilane and so forth; and trialkoxy silanes such as methyltrimethoxy silane, methyltriethoxy silane, methyltripropoxy silane, methyltributoxy silane, ethyltrimethoxy silane, ethyltriethoxy silane, n-propyltrimethoxy silane, n-propyltriethoxy silane, isopropyltrimethoxy silane, isopropyltriethoxy silane and so forth. In addition, as alkoxy silane partial condensate (B), the foregoing listed can be used without any particular limitation, but in the case of using at least two kinds among the listed in mixture, preferable is a synthesis obtained by employing at least 70 mol % of alkoxy silane partial condensate (B), based on the total constituting alkoxy silane monomer. Incidentally, when the content of a silane moiety contained in a polyurethane resin-silica hybrid is set to 1.0-30.0% by weight, very stable adhesiveness results.

Alkoxy silane partial condensate (B) is, for example, represented by following Formula (b) or Formula (c).



Formula (b) 25

In Formula (b), R<sup>1</sup> represents a lower alkyl group, an aryl group or an unsaturated fatty group which may have a functional group combined directly with a carbon atom, and R<sup>2</sup> represents a methyl group or an ethyl group. R<sup>2</sup>'s each may be the same or be different.



Formula (c)

R<sup>2</sup> in Formula (c) is the same R<sup>2</sup> as in Formula (b).

Examples of the method of the resin layer include a dipping method, a spray method, a roll coat method and a hand-varnishing coat method in consideration of viscosity of the resin component constituting a resin layer, but these forming methods are not limited in the present invention.

#### (Surface Layer)

On the other hand, a silicone copolymerization urethane resin employed for the surface layer can be synthesized with polyisocyanate which is at least difunctional, and a compound having in a molecule a silicone moiety containing a hydroxyl group which is at least difunctional. Preferably usable in the present invention is one having a JIS A hardness of 60-90° and a 100% modulus of 5×10<sup>6</sup>-30×10<sup>6</sup> Pa.

This silicone copolymerization urethane resin is not specifically limited, but those disclosed in Japanese Patent Examined Publication No. 7-33427 are usable.

Disclosed is a method of producing a polyurethane based resin via reaction of a polyol component, a polyisocyanate component and a chain extender component if desired, wherein a part of polyol is a copolymer of an active hydrogen-containing siloxane compound and lactones.

In order to obtain a polyurethane based resin via reaction of a polyol component, a polyisocyanate component and a chain extender component if desired, the polyurethane based resin is prepared by using a copolymer of an active hydrogen-containing siloxane compound and lactones. Examples of active hydrogen-containing siloxane compounds preferably usable in the present invention include the following compounds.

#### (1) Amino Modified Siloxane



(1-1)



(1-2)



(1-3)



(1-4)



(1-5)



(1-6)



(1-7)

#### (2) Epoxy Modified Siloxane



(2-1)



(2-2)



The above-described epoxy compound can be used by 30 having an active hydrogen at the terminal via reaction with polyol, polyamine, polycarboxylic acid or such.

(3) Alcohol Modified Siloxane



(5) Carboxyl Modified Siloxane



(3-5)

The above active hydrogen-containing siloxane compounds are siloxane compounds preferably usable in the present invention, and the present invention is not particularly limited thereto. Other siloxane compounds together with the above-described siloxane compounds are commercially available, and any of these is usable in the present invention. Incidentally, after monofunctional compounds are polymerized with lactones, the above-described siloxane compound can be incorporated into polyurethane via reaction with terminal NCO polyurethane.

(3-6)

In the present invention, lactones reacted with an active hydrogen-containing siloxane compound may possess substituents, the substituents are alkyl groups, aryl groups and so forth having 1-5 carbon atoms, and these each may be the same or different.

Preferably usable examples thereof include various monoalkyl- $\epsilon$ -caprolactones such as  $\epsilon$ -caprolactone, monoethyl- $\epsilon$ -caprolactone, monoethyl- $\epsilon$ -caprolactone, monopropyl- $\epsilon$ -caprolactone and monododecyl- $\epsilon$ -caprolactone; dialkyl- $\epsilon$ -caprolactones in which 2 alkyl groups each are substituted by other carbon atoms without bonding to carbon atoms at the  $\epsilon$ -positions. Also usable are alkoxy- $\epsilon$ -caprolactones such as trialkyl- $\epsilon$ -caprolactone and ethoxy- $\epsilon$ -caprolactone, or lactones such as cycloalkyl- $\epsilon$ -caprolactone, aryl- $\epsilon$ -caprolactone and aralkyl- $\epsilon$ -caprolactone like cyclohexyl, phenyl- $\epsilon$ -caprolactone, benzyl- $\epsilon$ -caprolactone in which carbon atoms at the  $\epsilon$ -positions in a lactone ring are not disubstituted, and other 2 or 3 carbon atoms are substituted by 3 alkyl groups.

As for the foregoing siloxane compound and the above-described caprolactone, they are mixed, and reacted under nitrogen stream at 150-200°C. for several hours to several 10 hours, employing an appropriate catalyst to obtain a siloxane modified poly caprolactone copolymer. They are reacted in any reaction ratio, but for the purpose of the present invention, they are preferably possible to be reacted in the proportion of 10-80 parts by weight of siloxane compound to 100 parts by weight of caprolactone. In the case of a consumption amount of the siloxane compound being too small, it is not preferred that insufficient non-adhesiveness and blocking resistance of the resulting polyurethane based resin are generated. Further, in the case of a consumption amount of the siloxane compound being excessive, it is not desired that transparency of the polyurethane based resin is lowered.

Further, usable is an intermediate layer obtained via reaction of the above-described copolymer with the after-mentioned polyisocyanate in such a way that at least one of a hydroxyl group in the copolymer and an isocyanate in the polyisocyanate group is left over. Similarly to the foregoing intermediate layer, for example, also usable is an intermediate layer obtained via reaction of a difunctional copolymer with polyfunctional polyisocyanate in an isocyanate group rich amount, or on the contrary, in a reactive group (in the copolymer) rich amount.

Further, polyester polyol and the like obtained via reaction of a copolymer with a polycarboxylic acid are similarly usable.

Any of commonly known polyurethane polyols is usable as the polyol employed in combination with the foregoing siloxane modified polycaprolactone copolymer, and preferable examples thereof include those having a number average molecular weight of 300-4000, and having a hydroxyl group as a terminal group such as polyethylene adipate, polyethylene propylene adipate, polyethylenebutylene adipate, polydiethylene adipate, polybutylene adipate, polyethylene succinate, polybutylene succinate, polyethylene sebacate, polybutylene sebacate, polytetramethylene ether glycol, poly- $\epsilon$ -caprolactone diol, polyhexamethylene adipate, carbonate polyol and polypropylene glycol, or those containing an appropriate amount of a polyoxyethylene chain in the above-described polyol.

Any of commonly known organic polyisocyanates is usable, but preferably usable examples thereof include 4,4'-diphenylmethane diisocyanate (MDI), water-added MDI, isophorone diisocyanate, 1,3-xylylene diisocyanate, 1,4-xylylene diisocyanate, 2,4-tolylene diisocyanate, 2,6-tolylene diisocyanate, 1,5-naphthalene diisocyanate, m-phenylene

diisocyanate and p-phenylene diisocyanate, or also usable is an urethane prepolymer obtained via reaction in such a way that low molecular weight polyol and polyamine together with these organic polyisocyanates are to be terminal isocyanates.

Any of commonly known chain extenders is usable, but preferably usable examples thereof include ethylene glycol, propylene glycol, diethylene glycol, 1,4-butanediol, 1,6-hexanediol, ethylenediamine, 1,2-propylenediamine, trimethylenediamine, tetramethylenediamine, hexamethylenediamine, decamethylene diamine, isophorone diamine, m-xylylene diamine, hydrazine, water and so forth.

Of these polyurethane based resins obtained from the foregoing material, a polyurethane based resin with the content of siloxane-caprolactone copolymer segment being 10-80% by weight, based on a polyurethane based resin molecule is specifically preferable. In the case of the content of less than 10% by weight, insufficient non-adhesiveness and blocking resistance are to be generated. In the case of the content exceeding 80% by weight, the resulting polyurethane based resin also exhibits insufficient transparency and flexibility. Further, a polyurethane based resin having a number average molecular weight of 20,000-500,000 is preferable, and that of 20,000-260,000 is more preferable.

Further, in the present invention, a polyurethane based resin having at least one released isocyanate group is produced via reaction of the above-described copolymer with polyisocyanate in isocyanate richness, and the resulting is used in combination with a coated film-forming resin to be utilized as a modifying agent.

A polyurethane based resin of the present invention containing the above-described siloxane-caprolactone copolymer segment can be prepared by a commonly known method. These polyurethane based resins may be prepared in a solventless process, or in an organic solvent, but the preparation in an organic solvent is of advantage in view of a process conducted in this case, since the resulting solution can be utilized for many purposes.

Examples of such the organic solvent preferably employed include that methyl ethyl ketone, methyl-n-propyl ketone, methyl isobutyl ketone, diethyl ketone, methyl formate, ethyl formate, propyl formate, methyl acetate, ethyl acetate, are butyl acetate, acetone, cyclohexane, tetrahydrofuran, dioxane, methanol, ethanol, isopropyl alcohol, butanol, toluene, xylene, dimethylformamide, dimethylsulfoxide, perchloroethylene, trichloroethylene, methylcellosolve, butylcellosolve, and cellosolve acetate.

#### (Effective Action of Surface Layer Resin)

Provided is a silicone polymerization polyurethane resin exhibiting excellent non-adhesiveness, blocking resistance and flexibility, together with excellent transparency by introducing a siloxane-caprolactone copolymer segment into a polyurethane based resin.

#### (Volume Resistance of Developing Roller)

Conductivity of a developing roller is possible to be evaluated via volume resistivity (called volume resistance or volume resistance value). The volume resistivity can be measured by a commonly known method.

In the present invention, it is assumed that appropriate conductivity appears when the developing roller volume resistivity measured by the following method is  $1 \times 10^2$  to  $1 \times 10^9$  W·cm. A developing roller volume resistivity of  $1 \times 10^3$  to  $1 \times 10^8$  W·cm is specifically preferable. The reason is that charge generated on the developing roller surface is appropriately

## 15

leaked, and the leakage current is appropriately controlled when the developing roller volume resistivity is in the above-described range.

The volume resistivity can be measured by a metal roller electrode method employing a typically known apparatus as shown in FIG. 5.

That is, stainless electrode roller 101 is brought into contact with developing roller 1, and pressed with a load of 9.8 N together with electrode roller 101 own weight. While rotating the roller in this situation, a voltage of +100 V is applied to an end of developing roller 1 to measure an electric current value. The developing roller volume resistivity is determined by using following Formula (1).

$$R=V/I$$

Formula (1)

## (Measuring Conditions)

Measurement environment: 23° C. and 57 RH %

Applied voltage: +100 V

Roller rotation speed: 27 rpm

Electrode roller load: 9.8 N (including electrode roller own weight)

Effective width of electrode roller: 230 mm (30 mm in diameter)

Measured item: Current value (applied voltage: a mean value after 5 seconds)

## [Preparation of Developing Roller]

The developing roller of the present invention, for example, can be produced as described below.

First, each component of the above-described elastic layer (base rubber layer) 3-forming material is kneaded with a kneader or such to prepare the elastic layer 3-forming material. After shaft 2 made of metal is set to a hollow portion of a cylindrical die, and the above elastic layer 3-forming material is cast-molded into a spacing gap between above cylindrical die 10 and shaft 2, the die is covered and heated to crosslink the elastic layer 3-forming material. Formwork removal from the above cylindrical die is subsequently conducted to form elastic layer 3 on the outer circumferential surface of shaft 2. The resulting in which the elastic layer is formed on the outer circumferential surface of the shaft is designated as "base roller".

On the other hand, a resin layer (intermediate layer) 4 forming material is mixed with an organic solvent, and dissolved to prepare a solution. Subsequently, inorganic or organic particles may be added into the resulting solution, and may be mixed to prepare the intermediate layer 4 forming solution. In this case, the above-described particles are not dissolved in a conventional solvent since these particles are rigid, but are dispersed in the solvent.

A surface layer 5 forming solution is also prepared by mixing a surface layer 5 forming material with an organic solvent.

After this, the above-described resin layer 4 forming solution is coated on the outer circumferential surface of elastic layer 3 of the above-described base roller. This coating method is not particularly limited, and a commonly known method such as a dipping method, a spray method or a roller coat method can be employed. A solvent in the above-described resin layer 4 forming solution is subsequently removed to form the resin layer via drying and heat treatment after coating (vulcanizing treatment at 120-200° C. for 20-90 minutes). And then, the above-described surface layer 5 forming solution is coated on the outer circumferential surface of above-described resin layer 4. A commonly known method as the coating method can be employed similarly to the case of the above-described resin layer 4 forming solution. A solvent

## 16

in the above-described surface layer 5 forming solution is subsequently removed to form surface layer 5 via drying and heat treatment after coating (vulcanizing treatment at 120-200° C. for 20-90 minutes). In this way, a developing roller having a structure of at least two layers as shown in FIG. 1 can be prepared. As to this developing roller, elastic layer 3 preferably has a thickness of 1-10 mm, and more preferably has a thickness of 2-6 mm. Resin layer 4 preferably has a thickness of 3-30 µm, and more preferably has a thickness of 5-20 µm. The thickness of surface layer 5 is preferably set to 3-30 µm, and more preferably set to 5-20 µm. The thickness of each layer including above-described intermediate layer 4 can be measured via microscope observation after obtaining a cut plane sample including surface layer 5, intermediate layer 4 and elastic layer 3 in the developing roller.

In addition, a developing roller having a three-layer structure was shown in FIG. 1 as an example of developing roller of the present invention, but the layer structure formed around the outer circumference of shaft 2 is not necessarily a structure of three layers, and a structure of the appropriate number of layers such as at least three layers between elastic layer 3 and surface layer 5 may be formed as roller usage. An outermost surface layer among resin layers is also called a surface layer.

## (Developer)

Toner of the present invention may also be prepared via a pulverizatio/classification process (via a so-called polymerization process). In the case of conducting the polymerization process, a process of salting-out/fusing resin particles is preferable.

## (Monomer)

As a polymerizable monomer, a radically polymerizable monomer is employed as a mandatory component, and a crosslinking agent is usable, if desired. It is also preferable to contain at least one kind of radically polymerizable monomers having the following acidic group or basic group.

## (1) Radically Polymerizable Monomer

Radically polymerizable monomers are not particularly limited, and commonly known radically polymerizable monomers are usable. These monomers can be used singly or in combination with at least two kinds in order to satisfy desired properties.

Specifically, usable examples thereof include an aromatic vinyl monomer, a (meth)acrylic acid ester based monomer, a vinyl ester based monomer, a vinyl ether based monomer, a monoolefin based monomer, a diolefin based monomer and a halogenated olefin based monomer.

Examples of the aromatic vinyl monomer include a styrene based monomer such as styrene, o-methylstyrene, m-methylstyrene, p-methylstyrene, p-methylstyrene, p-phenylstyrene, p-chlorostyrene, p-ethylstyrene, p-n-butylstyrene, p-tert-butylstyrene, p-n-hexylstyrene, p-n-octylstyrene, p-n-nonylstyrene, p-n-decylstyrene, p-n-dodecyl styrene, 2,4-dimethylstyrene or 3,4-dichlorostyrene, and a derivative thereof.

Examples of the ester acrylate based monomer include methyl acrylate, ethyl acrylate, butyl acrylate, acrylic acid-2-ethylhexyl, cyclohexyl acrylate, phenyl acrylate, methyl methacrylate, ethyl methacrylate, butyl methacrylates, hexyl methacrylate, methacrylic acid-2-ethylhexyl, b-hydroxy-acrylic acid ethyl, g-aminoacrylic acid propyl, stearyl methacrylate, dimethylaminoethyl methacrylate and diethylaminoethyl methacrylate.

Examples of the vinyl ester based monomer include vinyl acetate, vinyl propionate, vinyl benzoate and so forth.

Examples of the vinyl ether based monomer include vinyl-methyl ether, vinyl-ethyl ether, vinyl-isobutyl ether, vinyl-phenyl ether and so forth.

Examples of the monoolefin based monomer include ethylene, propylene, isobutylene, 1-butene, 1-pentene, 4-methyl-1-pentene and so forth.

Examples of the diolefin based monomer include butadiene, isoprene, chloroprene, and so forth.

Examples of the halogenation olefin based monomer include vinyl chloride, vinylidene chloride, vinyl bromide and so forth.

#### (2) Crosslinking Agent

A radical polymerizable crosslinking agent may be added as a crosslinking agent in order to improve toner characteristics. A crosslinking agent having at least two unsaturated bonds such as divinylbenzene, divinylnaphthalene, divinylether, diethylene glycol methacrylate, ethylene glycol dimethacrylate, polyethylene glycol dimethacrylate or diallyl phthalate is provided as the radically polymerizable crosslinking agent.

#### (3) Radically Polymerizable Monomer Having an Acidic Group or Radically Polymerizable Monomer Having a Basic Group

Usable examples of the radically polymerizable monomer having an acidic group or the radically polymerizable monomer having a basic group include a carboxyl group-containing monomer, a sulfonic acid group-containing monomer, and amine based compounds such as primary amine, secondary amine, tertiary amine and quaternary ammonium salt.

Examples of the radically polymerizable monomer having an acidic group include an acrylic acid, a methacrylic acid, a fumaric acid, a maleic acid, an itaconic acid, a cinnamic acid, a maleic acid monobutyl ester, a maleic acid mono-octyl ester and so forth.

Examples of the sulfonic acidic group-containing monomer include styrene sulfonic acid, allylsulfosuccinic acid, allylsulfosuccinic acid octyl and so forth.

These may be a structure of alkaline metal salt such as sodium or potassium, or a structure of alkaline earth metal salt such as calcium.

Examples of the radically polymerizable monomer having a basic group include amine based compounds such as dimethylamino ethyl acrylate, dimethylamino ethyl methacrylate, diethylaminoethyl acrylate, diethylaminoethyl methacrylate and quarternary ammonium salts of the above-described four compounds, and 3-dimethylaminophenyl acrylate, 2-hydroxy-3-methacryloxypropyltrimethyl ammonium salt, acrylamide, N-butylacrylamide, N,N-dibutylacrylamide, piperidylacrylamide, methacrylamide, N-butyl-methacrylamide, N-octadecylacrylamide; and vinylpyridine, vinyl pyrrolidone, vinyl-N-methylpyridinium chloride, vinyl-N-ethylpyridinium chloride, N,N-diallylmethyl ammonium chloride, and N,N-diallylethyl ammonium chloride.

As for a radically polymerizable monomer of the present invention, the content of the radically polymerizable monomer having an acidic group or the radically polymerizable monomer having a basic group is preferably 0.1-15% by weight, based on the total radically polymerizable monomer, and more preferably 0.1-10% by weight, though depending on the properties of a radically polymerizable crosslinking agent.

#### (Chain Transfer Agent)

Commonly known chain transfer agents are usable for the purpose of adjusting a molecular weight.

Chain transfer agents are not particularly limited, and usable examples thereof include octylmercaptan, dodecylmercaptan, tert-dodecylmercaptan, n-octyl-3-mercaptopropionic acid ester, carbon tetrabromide and styrene dimmer.

#### (Polymerization Initiator)

A radical polymerization initiator of the present invention is suitably usable, provided that it is water-soluble. Examples thereof include persulfates such as potassium persulfate, ammonium persulfate and so forth; azo based compounds such as 4,4'-azobis-4-cyano valeric acid, a salt thereof and 2,2'-azobis(2-amidinopropane) salt; and a paroxide compound.

Further, the above-described radically polymerizable monomer can be a redox based initiator in combination with a reducing agent, if desired. It is expected that polymerization is activated by using the redox based initiator, the polymerization temperature can be lowered, and the polymerization time can further be shortened.

The polymerization temperature may be optionally selected if it is at least the minimum radical generation temperature of a polymerization initiator, but a temperature range of 50-90° C. is usable. Polymerization is also possible to be done at room temperature or slightly more by employing a polymerization initiator working at normal temperature in combination with hydrogen peroxide-reducing agent (ascorbic acid and so forth).

#### (Surfactant)

In order to conduct polymerization employing the foregoing radically polymerizable monomer, oil droplets are desired to be dispersed in an aqueous medium by using a surfactant. Surfactants usable in this case are not particularly limited, but ionic surfactants listed below are usable.

Examples of the ionic surfactant include sulfonate such as dodecyl benzene sulfonic acid sodium, arylalkyl polyether-sulfonic acid sodium, 3,3-disulphone diphenylurea-4,4-diazo-bis-amino-8-naphthol-6-sodium sulphonate, ortho-carboxy benzene-azo-dimethylaniline or 2,2,5,5-tetramethyl-triphenyl methane-4,4-diazo-bis-β-naphthol-6-sodium sulfonate; sulfuric ester salt such as sodium dodecyl sulfate, sodium tetradecyl sulfate, pentadecyl sodium sulfate or sodium octylsulphate; and fatty acid salt such as sodium oleate, lauric acid sodium, capric acid sodium, caprylic acid sodium, caproic acid sodium, stearic acid potassium or oleic acid calcium.

Examples of the nonionic surfactant also include polyethylene oxide, polypropylene oxide, combination of polypropylene oxide and polyethylene oxide, ester of polyethyleneglycol and higher fatty acid, alkylphenol polyethylene oxide, ester of higher fatty acid and polyethyleneglycol, ester of higher fatty acid and polypropylene oxide, and sorbitan ester.

In the present invention, these are mainly employed for an emulsifying agent in emulsion polymerization. They may be used in other processes or other purpose of use.

#### (Colorant)

Inorganic pigment, organic pigment and dye are usable as a colorant.

Commonly known pigments are usable as the inorganic pigment. Specific inorganic pigments are exemplified below.

Carbon black such as furnace black, channel black, acetylene black, thermal black or lamp black is exemplified as a black pigment, and magnetic powder made of magnetite or ferrite is also employed.

These inorganic pigments can be used singly, or plural kinds can be used in combination, if desired. The addition

19

amount of the pigment is 2-20% by weight, based on the weight of polymer, and preferably 3-15% by weight.

Commonly known organic pigments or dyes are usable as the organic pigment and the dye. The following examples of organic pigments and dyes are specifically listed.

Examples of pigments for magenta or red include C. I. Pigment Red 3, C. I. Pigment Red 3, C. I. Pigment Red 5, C. I. Pigment Red 6, C. I. Pigment Red 7, C. I. Pigment Red 15, C. I. Pigment Red 16, C. I. Pigment Red 48:1, C. I. Pigment Red 53:1, C. I. Pigment Red 57:1, C. I. Pigment Red 122, C. I. Pigment Red 123, C. I. Pigment Red 139, C. I. Pigment Red 144, C. I. Pigment Red 149, C. I. Pigment Red 166, C. I. Pigment Red 177, C. I. Pigment Red 178, C. I. Pigment Red 222 and so forth.

Examples of pigments for orange or yellow include C. I. Pigment Orange 31, C. T. Pigment Orange 43, C. I. Pigment Yellow 12, C. I. Pigment Yellow 13, C. I. Pigment Yellow 14, C. I. Pigment Yellow 15, C. T. Pigment Yellow 17, C. I. Pigment Yellow 93, C. I. Pigment Yellow 94, C. I. Pigment Yellow 138, C. I. Pigment Yellow 180, C. I. Pigment Yellow 185, C. I. Pigment Yellow 155, C. I. Pigment Yellow 156 and so forth.

Examples of pigments for green or cyan include C. I. Pigment Blue 15, C. T. Pigment Blue 15:2, C. T. Pigment Blue 15:3, C. I. Pigment Blue 16, C. I. Pigment Blue 60, C. I. Pigment Green 7 and so forth.

Further, examples of dyes include C. I. Solvent Red 1, C. T. Solvent Red 49, C. I. Solvent Red 52, C. I. Solvent Red 58, C. I. Solvent Red 63, C. I. Solvent Red 111, C. I. Solvent Red 122, C. I. Solvent Yellow 19, C. I. Solvent Yellow 44, C. I. Solvent Yellow 77, C. I. Solvent Yellow 79, C. T. Solvent Yellow 81, C. I. Solvent Yellow 82, C. I. Solvent Yellow 93, C. I. Solvent Yellow 98, C. I. Solvent Yellow 103, C. I. Solvent Yellow 104, C. I. Solvent Yellow 112, C. I. Solvent Yellow 162, C. I. Solvent Blue 25, C. I. Solvent Blue 36, C. I. Solvent Blue 60, C. I. Solvent Blue 70, C. I. Solvent Blue 93, C. I. Solvent Blue 95 and so forth.

These organic pigments and dyes can be used singly, or plural kinds can be used in combination, if desired. The addition amount of the pigment is 2-20% by weight, based on the weight of polymer, and preferably 3-15% by weight.

#### (Wax)

Toner usable in the present invention may contain wax, and the structure and composition of wax are not particularly limited. Usable examples thereof include low molecular weight polyolefin wax such as polypropylene or polyethylene; paraffin wax; Fischer-tropush wax, ester wax and so forth.

The addition amount is 1-30% by weight, based on the total weight of toner, preferably 2-20% by weight, and more preferably 3-15% by weight.

The toner usable in the present invention is preferably a toner wherein wax dissolved in a monomer is dispersed in water and polymerized to form resin particles in which an ester based compound is included, and to salt-out/fuse them with colorant particles.

#### (Manufacturing Process)

Toner usable in the present invention is preferably produced by a polymerization method comprising the steps of preparing resin particles including wax via a polymerization method after dispersing a monomer solution, in which wax is dissolved, in an aqueous medium; fusing resin particles in the aqueous medium employing the foregoing resin particle dispersion; removing a surfactant and so forth by filtrating the resulting particles from the aqueous medium; drying the resulting particles; and further adding external additives and so forth into particles obtained after drying. Resin particles

20

herein may also be colored particles. Uncolored particles are also usable as resin particles. In this case, colored particles are prepared via a fusing process in an aqueous medium after adding a colorant particle dispersion into a resin particle dispersion.

It is preferable that resin particles prepared via a polymerization process are specifically utilized as a fusing process to conduct salting-out/fusing. Further, in the case of employing uncolored resin particles, resin particles and colorant particles can be subjected to salting-out/fusing in an aqueous medium.

Further, particles are not limited to a colorant and wax, but a charge control agent constituting the toner as a component can also be added in the present process as the particles.

Incidentally, the aqueous medium is water as a principal component, and has the content of water being at least 50% by weight. Water-soluble organic solvents other than water are also provided, and examples thereof include methanol, ethanol, isopropanol, butanol, acetone, methylethyl ketone, tetrahydrofuran and so forth.

As a preferable polymerization method of preparing toner usable in the present invention, provided can be a radical polymerization method in which a water-soluble polymerization initiator is added into a dispersion obtained by mechanically oil-droplet-dispersing a monomer solution in which wax was dissolved in a monomer, in an aqueous medium in which a surfactant of the critical micelle concentration or less is dissolved. In this case, an oil-soluble polymerization initiator may also be added into a monomer, and be usable.

The homogenizer for dispersing oil droplets is not specifically limited, but Cleamix, an ultrasonic homogenizer, a mechanical homogenizer, Manton-Gaulin, a pressure type homogenizer and so forth, for example, can be listed.

As is described before, the colorant itself may be used by modifying the surface. The surface modification method of colorants is a method in which colorants are dispersed in a solvent, and temperature is increased to accelerate a chemical reaction after adding a surface modification agent into the resulting solution. After terminating the reaction, the resulting solution is filtrated, washing and filtrating processes are repeatedly conducted with the same solvent, and then a drying process is carried out to obtain a pigment subjected to a treatment employing the surface modification agent.

There is a process in which colorant particles can be prepared by dispersing a colorant in an aqueous medium. This dispersion treatment is carried out in a state where the surfactant concentration is arranged to at least critical micelle concentration (CMC) in water.

Although the homogenizer employed during pigment dispersion is not specifically limited, preferably listed are Cleamix, an ultrasonic homogenizer, a mechanical homogenizer, a pressure homogenizer such as Manton-Gaulin or a pressure type homogenizer, a sand grinder, and a media type homogenizer such as a Getzmann mill or a diamond fine mill.

The foregoing surfactant is usable as a surfactant utilized here.

The salting-out/fusing process is a process wherein a salting-out agent containing an alkali metal salt or an alkaline earth metal salt is added into water, in which resin particles and colorant particles exist, as a coagulant having at least the critical coagulation concentration, and subsequently the resulting solution is heated to a temperature of at least the glass transition point of the resin particles to conduct salting-out and fusing simultaneously.

Examples of the alkali metal salt and alkaline earth metal salt usable as salting-out agents include: salts of alkali metals such as lithium, potassium and sodium; and salts of alkaline

earth metals such as magnesium, calcium, strontium and barium. Of these, potassium, sodium, magnesium, calcium and barium are preferable. Listed as components constituting the salt may be, for example, chlorine salt, bromine salt, iodine salt, carbonate and sulfate.

(Other Additives)

A material as a toner substance in which various functions can be given, other than a resin, a colorant and wax is usable for toner. A charge control agent and so forth are specifically provided. These components can be added via various processes such as a process of including these inside toner after adding resin particles and colorant particles simultaneously at the stage of the foregoing salting-out/fusing, a process of adding these into the resin particle itself, and so forth.

Similarly, usable are commonly known various charge control agents which are water-dispersible. Examples thereof include a nigrosine based dye, a metal salt of a naphthenic acid or a higher fatty acid, alkoxylated amine, a quaternary ammonium salt compound, an azo based metal complex, and a salicylic acid metal salt or its metal complex.

(External Additives)

So-called external additives can be employed for toner usable in the present invention, and added to improve fluidity and an electrostatic property, and to enhance cleaning capability. These external additives are not particularly limited, and various inorganic and organic particles, and lubricants are usable.

Commonly known particles are usable as inorganic particles. Specifically usable are silica, titanium and alumina particles preferably having a number average primary particle diameter of 5-500 nm. These inorganic particles are preferably hydrophobic.

Examples of silica particles include commercially available products such as R-805, R-976, R-974, R-072, R-812 and R-809 produced by Nippon Aerosil Co., Ltd.; commercially available products such as HVK-2150 and H-200 produced by Höchst; commercially available products such as TS-720, TS-530, TS-610, H-5 and MS-5 produced by Cabot corporation.

Examples of titanium particles include commercially available products such as T-805 and T-604 produced by Nippon Aerosil Co., Ltd.; commercially available products such as MT-100S, MT-100B, MT-500BS, MT-600, MT-600SS and JA-1 produced by Tayca Corporation; commercially available products such as TA-300SI, TA-500, TAF-130, TAF-510, TAF-510T produced by Fuji Titanium Industry Co., Ltd.; and commercially available products such as IT-S, IT-OA, IT-OB and IT-OC produced by Idemitsu Kosan Co., Ltd.

Examples of alumina particles include commercially available products such as RFY-C and C-604 produced by Nippon Aerosil Co., Ltd.; and commercially available products such as TT-55 and so forth produced by Ishihara Sangyo Kaisha, Ltd.

Spherical organic particles having a number average primary particle diameter of approximately 10 -2000 nm are usable as organic particles. These usable organic particles are formed from a homopolymer or its copolymer of styrene, methylmethacrylate or such.

As the lubricant, provided are higher fatty acid metal salts such as a stearic acid zinc salt, a stearic acid aluminum salt, a stearic acid copper salt, a stearic acid magnesium salt, a stearic acid calcium salt and so forth; an oleic acid zinc salt, an oleic acid manganese salt, an oleic acid iron salt, an oleic acid copper salt, an oleic acid magnesium salt and so forth; a palmitic acid zinc salt, a palmitic acid copper salt, a palmitic

acid magnesium salt, a palmitic acid calcium salt and so forth; a linolic acid zinc salt, a linolic acid calcium salt and so forth; and a recinoleic acid zinc salt, a recinoleic acid calcium salt and so forth.

5 The addition amount of these external additives is preferably 0.1-5% by weight, based on the weight of toner.

Examples of commonly known mixers usable as a method of adding external additives include a tabular mixer, a Henschel mixer, a nauter mixer and a V-shaped mixer. In addition, 10 the toner particle diameter is preferably 3-8  $\mu\text{m}$  in terms of the volume-based median diameter measured employing "Multisizer 3, manufactured by Beckman Coulter Co., Ltd."

[Image Forming Method]

15 An image forming apparatus with non-magnetic single component development in the present invention comprises a developing roller, a toner layer regulating member and an auxiliary toner supply member, and it is usual that auxiliary toner supply member is brought into contact with the developing roller, and the toner layer regulating member is also brought into contact with the toner conveying member. This is a process in which the thin-layered non-magnetic toner is supplied onto the electrostatic latent image forming body surface to develop the latent image, employing the apparatus.

20 The toner layer regulating member exhibits functions which uniformly apply toner onto the toner conveying member and in addition which provides frictional electrification. Specifically employed as the members are elastic bodies such as urethane rubber and metal panels. The toner layer regulating member is brought into contact with the toner conveying member, whereby a thin toner layer is formed on the toner conveying member. The thin toner layer, as described herein, 25 refers to a layer in the state that a toner layer is composed of at most 10 layers in a developing region and preferably at most 5 layers. The toner layer regulating member is preferably brought into contact with the toner conveying member at a pressure of 100 mN/cm to 5 N/cm, and more preferably at a pressure of 200 mN/cm to 4 N/cm. In the case of this pressure being less than 100 mN/cm, toner conveyance becomes fluctuated, resulting easily in uneven toner conveyance, whereby 30 white a problem caused by white streak tends to occur. On the other hand, in the case of this pressure exceeding 5N/cm, shortage of toner supply, and deformation and crushing of toner tend to occur. The toner conveying member preferably has a diameter of 10-50 mm.

35 The auxiliary toner supply member is a unit to uniformly supply toner to the developing roller. Employed as the units may be water wheel-shaped rollers fitted with stirring blades or sponge-shaped rollers. In the present invention, the diameter with respect to the toner supply member is preferably in the range of 0.2-1.5 times. When this diameter is too small, toner supply becomes insufficient. On the other hand, when this diameter is too large, the toner supply becomes excessive. Both cases tend to result in streaking image problems.

40 Specific examples of the electrostatic latent carrier include a selenium inorganic photoreceptor or an arsenic selenium inorganic photoreceptor, an amorphous silicon photoreceptor and an organic photoreceptor. Of these, an organic photoreceptor is preferable, but an organic photoreceptor having a charge generation layer and a charge transfer layer is more preferable.

45 Next, the developing device (developing unit) employed in an image forming method of the present invention will be specifically explained.

50 FIG. 4 is a schematic cross-sectional illustration of a developing device employed in an image forming method of the present invention.

In FIG. 4, non-magnetic single component toner **16**, stored in toner tank **17**, is forcibly conveyed and supplied onto sponge roller **14** as an auxiliary toner supply member, employing stirring blade **15** as the auxiliary toner supply member. Toner adhered on the sponge roller is conveyed to developing roller **1** as a toner conveying member, via rotation in the arrowed direction of sponge roller **14**, and is electrostatically and physically adsorbed onto its surface due to friction with developing roller **1**. On the other hand, the toner adhered onto developing roller **1**, as described above, is subjected to uniformly thin-layering by rotation of developing roller **1** in the arrowed direction, together with flexible steel blade **13** as a toner layer thickness regulating member, and is also subjected to frictional electrification. The thin toner layer formed on developing roller **1** comes into contact with or approaches the surface of electrophotographic drum (photoreceptor) **11**, whereby a latent image is developed.

Incidentally, the structure of a developing device employed in the present invention is not particularly limited to the structure shown in FIG. 4.

A so-called contact heating process can be provided as a preferable fixing process usable in the present invention. Specific examples of the contact heating process include a heat pressure fixing process, and further a heat roller fixing process and a pressing contact heat-fixing process in which a rotary pressing member including a fixed heating body is employed for fixing.

The heat-roll fixing process is operated by an upper roller and a lower roller, wherein the upper roller contains a heat source inside the metal cylinder made of iron or aluminum covered with tetrafluoroethylene, polytetrafluoroethylene-perfluoroalkoxyvinyl ether copolymer or such, and the lower roller is made of a silicone rubber or others. A linear heater is provided as a heat source and is usually employed to heat the upper roller to a surface temperature of about 120-200° C. In the fixing section, pressure is applied between the upper roller and lower roller to deform the lower roller, whereby a so-called nip is formed. The nip width is 1-10 mm, preferably 1.5-7 mm. The fixing linear speed is preferably 40-600 mm/sec. When the nip width is small, heat can not be applied uniformly, and uneven fixing will occur. If the nip width is large, resin fusion will be accelerated and the problem of excessive fixing offset will arise.

A fixing cleaning mechanism may be provided to be utilized. As to this process, it is possible to use a process of supplying silicone oil to a fixing upper roller or film, or a cleaning process employing a pad, a roller, a web or such impregnated with silicone oil.

In the present invention, also usable is a process in which a rotary pressing member including a fixed heating body is employed for fixing.

This fixing process is a pressing contact heat-fixing process in which fixing is conducted with a fixed heating body and a pressing member by which contact-pressing facing the heating body is applied, and a recording material is attached to the heating body via a film.

This pressing contact heat-fixing device is equipped with a heating body having a smaller heat capacity than that of a conventional heating body, and has a heating portion in the form of lines at a right angle to the passing direction of the

recording material. The maximum temperature of the heating portion is usually 100-300° C.

## EXAMPLE

Next, the embodiments of the present invention will further be explained, referring to examples, but the present invention is not limited thereto.

Incidentally, "parts" in the description represents "parts by weight"

### (Preparation Example of Developing Roller)

Mixed and dispersed were 100 parts of X-34-424:A/B (silicone rubber, produced by Shin-Etsu Chemical Co., Ltd.) and 100 parts of X-34-387:A/B (silicone rubber, produced by Shin-Etsu Chemical Co., Ltd.), and 80 parts of Ketjen Black were further added into this to prepare elastic layer-forming material **1**.

### (Preparation Example 1 of Polyurethane Resin-Silica Hybrid Intermediate Layer-Forming Material)

Into a reactor fitted with a stirrer, a thermometer and a nitrogen gas-introducing tube, charged were 100 g of polycarbonate diol having a number average molecular weight of 2000 (PLACCEL CD220, produced by Daicel Chemical Industries, Ltd.) and 278 g of isophorone diisocyanate, the system was reacted under nitrogen gas stream at 100° C. for 6 hours to prepare a prepolymer having a released isocyanate value of 3.44%, and 548 g of methylethyl ketone was subsequently added into the resulting to prepare an even urethane prepolymer solution. Next, 1000 g of the above-described urethane prepolymer solution was added in the presence of a mixture composed of 71.8 g of isophorone diamine, 4.0 g of di-n-butylamine, 906 g of methylethyl ketone and 603 g of isopropyl alcohol, and the resulting was reacted at 50° C. for 3 hours. The resulting polyurethane resin solution {hereinafter, referred to as polyurethane resin (1A)} had a resin solid content of 30% by weight and an amine value of 1.2 KOHmg/g.

On the other hand, 1400 g of glycidol (EPIOL, produced by NOF Corporation) and 8957.9 g of a tetramethoxysilane partial condensate having a Si average number of 4 (Methyl Silicate -51, produced by Tama Chemicals Co., Ltd.) were charged into a reactor fitted with a stirrer, a diversion device, a thermometer and a nitrogen gas-introducing tube, and temperature was increased to 90° C. while stirring under nitrogen gas stream to react with an addition of 2.0 g of dibutyltin dilaurate as a catalyst. In the reaction, methanol was distilled away employing a diversion device, and the system was cooled when the amount reached about 630 g. Time consumed for cooling after increasing temperature was 5 hours. Next, approximately 80 g of methanol remaining in the system was removed at a reduced pressure of 13 kPa for 10 minutes to obtain epoxy group-containing alkoxy silane partial condensate (2A).

After 500 g of the foregoing polyurethane resin (1A) was increased to a temperature of 50° C., 10.95 g of the foregoing epoxy group-containing alkoxy silane partial condensate (2A) was added, and the resulting was reacted under nitrogen gas stream at 60° C. for 4 hours to prepare an alkoxy group-containing silane modified polyurethane resin.

Mixed and dispersed were 100 parts of the resulting alkoxy group-containing silane modified polyurethane resin and 30 parts of Ketjen Black (carbon black) to prepare intermediate layer (immediately below the surface layer)-forming material **1**.

In addition, the content of Si contained in the solid residue in the alkoxy group-containing silane modified polyurethane resin was 3.3% in silica weight conversion.

25

## (Preparation Example 2 of Polyurethane Resin-Silica Hybrid Intermediate Layer-Forming Material)

A polyurethane resin solution {hereinafter, referred to as polyurethane resin (1B)} was prepared in the same reaction as in preparation example 1, except that "PLACCEL CD220" was replaced by polyester polyol having a number average molecular weight of 2000 (Kurapol P2010, produced by Kuraray Co., Ltd.) in preparation example 1 of the intermediate layer-forming material. Polyurethane resin (1B) had a resin content of 30% and an amine value of 1.2 KOHmg/g.

Into the same reactor as in preparation example 1, charged were 250.0 g of glycidol and 2675.4 g of a tetramethoxysilane partial condensate having a Si average number of 10 (Methyl Silicate 56, produced by Tama Chemicals Co., Ltd.), and temperature was increased to 90° C. while stirring under nitrogen gas stream to react with an addition of 0.5 g of dibutyltin dilaurate as a catalyst. In the reaction, methanol was distilled away employing a diversion device, and the system was cooled when the amount reached about 125 g. Time consumed for cooling after increasing temperature was 6.5 hours. Next, approximately 5 g of methanol remaining in the system was removed at a reduced pressure of 13 kPa for 10 minutes to obtain epoxy group-containing alkoxy silane partial condensate (2B).

After 500 g of the foregoing polyurethane resin (1B) was increased to a temperature of 50° C., 17.75 g of the foregoing epoxy group-containing alkoxy silane partial condensate (2B) was added, and the resulting was reacted under nitrogen gas stream at 60° C. for 4 hours to prepare an alkoxy group-containing silane modified polyurethane resin.

Mixed and dispersed were 100 parts of the resulting alkoxy group-containing silane modified polyurethane resin and 30 parts of Ketjen Black (carbon black) to prepare intermediate layer (immediately below the surface layer)-forming material 2.

In addition, the content of Si contained in the solid residue in the alkoxy group-containing silane modified polyurethane resin was 6.0% in silica weight conversion.

## (Preparation Example 3 of Polyurethane Resin-Silica Hybrid Intermediate Layer-Forming Material)

Into the same reactor as in preparation example 1 of the intermediate layer-forming material, charged were 1000 g of "PLACCEL CD220" and 278 g of isophorone diisocyanate, the system was reacted under nitrogen gas stream at 100° C. for 6 hours to prepare a prepolymer having a released isocyanate value of 3.44%, and 548 g of methylethyl ketone was subsequently added into the resulting to prepare an even urethane prepolymer solution. Next, 1000 g of the above-described urethane prepolymer solution was added in the presence of a mixture composed of 77.6 g of isophorone diamine, 2.4 g of di-n-butylamine, 913 g of methylethyl ketone and 607 g of isopropyl alcohol, and the resulting was reacted at 50° C. for 3 hours. The resulting polyurethane resin solution {hereinafter, referred to as polyurethane resin (1C)} had a resin solid content of 30% by weight and an amine value of 2.4 KOHmg/g. After 500 g of the foregoing polyurethane resin (1C) was increased to a temperature of 50° C., 18.54 g of the foregoing epoxy group-containing alkoxy silane partial condensate (2A) obtained in preparation example 1 was added, and the resulting was reacted under nitrogen gas stream at 60° C. for 4 hours to prepare an alkoxy group-containing silane modified polyurethane resin.

Mixed and dispersed were 100 parts of the resulting alkoxy group-containing silane modified polyurethane resin and 30

26

parts of Ketjen Black (carbon black) to prepare intermediate layer (immediately below the surface layer)-forming material 3.

In addition, the content of Si contained in the solid residue in the alkoxy group-containing silane modified polyurethane resin was 6.4% in silica weight conversion.

## (Preparation Example 4 of Polyurethane Resin-Silica Hybrid Intermediate Layer-Forming Material)

10 Into the same reactor as in preparation example 1 of the intermediate layer-forming material, charged were 1000 g of "Kurapol P2010", 40 g of dimethylol butanoic acid and 342 g of isophorone diisocyanate, the system was reacted under nitrogen gas stream at 100° C. for 6 hours to prepare a prepolymer having a released isocyanate value of 3.28%, and 593 g of methylethyl ketone was subsequently added into the resulting to prepare an even urethane prepolymer solution. Next, 1000 g of the above-described urethane prepolymer solution was added in the presence of a mixture composed of 59.7 g of isophorone diamine, 9.9 g of di-n-butylamine, 897 g of methylethyl ketone and 599 g of isopropyl alcohol, and the resulting was reacted at 50° C. for 3 hours. The resulting polyurethane resin solution {hereinafter, referred to as polyurethane resin (1D)} had a resin solid content of 30% by weight and an amine value of 3.0 KOHmg/g. After 500 g of the foregoing polyurethane resin (1D) was increased to a temperature of 50° C., 18.54 g of the foregoing epoxy group-containing alkoxy silane partial condensate (2A) obtained in preparation example 1 was added, and the resulting was reacted under nitrogen gas stream at 60° C. for 4 hours to prepare an alkoxy group-containing silane modified polyurethane resin.

Mixed and dispersed were 100 parts of the resulting alkoxy group-containing silane modified polyurethane resin and 30 parts of Ketjen Black (carbon black) to prepare intermediate layer (immediately below the surface layer)-forming material 4.

In addition, the content of Si contained in the solid residue in the alkoxy group-containing silane modified polyurethane resin was 7.8% in silica weight conversion.

## (Preparation Example 1 of Silicone Copolymerization Polyurethane Resin Surface Layer-Forming Material)

45 Into a reactor fitted with a stirrer, a thermometer, a nitrogen gas-introducing tube and a reflux condenser, charged were 310 parts of  $\epsilon$ -caprolactone, 150 parts of alcohol modified siloxane (exemplified compound 3-3) and 0.05 parts of tetrabutyltitanate, and the system was reacted under nitrogen gas stream at 180° C. for 10 hours to prepare a polysiloxane-polyester copolymer having a number average molecular weight of 3030, an acidic value of 0.40 and a hydroxyl value of 37.

55 In a mixed solvent of 200 parts of methylethyl ketone and 100 parts of dimethylformamide, dissolved were 150 parts of the above-described copolymer and 27 parts of 1,4-butanediol, and then a solution obtained by dissolving 91 parts of water-added diphenylmethanediisocyanate (referred to also as water-added MDI or H12MDI) in 188 parts of dimethylformamide was gradually dripped while stirring at 60° C. After dripping was completed, the resulting was reacted at 80° C. for 6 hours to prepare a silicone copolymerization polyurethane resin solution of the present invention. This solution exhibited high transparency, accompanied with a viscosity of 35.5 Pa·s (25° C.) at a solid content of 35%.

60 Further, 100 parts of the resulting silicone copolymerization polyurethane resin, 30 parts of Ketjen Black (carbon black) and 40 parts of particles made of a crosslinked ure-

thane resin having a number average primary particle diameter of 20  $\mu\text{m}$  were mixed and dispersed to prepare surface layer-forming material 1.

(Preparation Example 2 of Silicone Copolymerization Polyurethane Resin Surface Layer-Forming Material)

In a mixed solvent of 200 parts of methylethyl ketone and 150 parts of dimethylformamide, dissolved were 75 parts of a copolymer of foregoing preparation example 1, 75 parts of polybutylene adipate having a number average molecular weight of 2000, an acidic value of 0.40 and a hydroxyl value of 56.0, and 27 parts of 1,4-butanediol, and then a solution obtained by dissolving 90 parts of MDI in 146 parts of dimethylformamide was gradually dripped while stirring at 60° C. After dripping was completed, the resulting was reacted at 80° C. for 6 hours to prepare a silicone copolymerization polyurethane resin solution of the present invention. This solution exhibited high transparency, accompanied with a viscosity of 31.2 Pa·s (25° C.) at a solid content of 35%.

Further, 100 parts of the resulting silicone copolymerization polyurethane resin, 30 parts of Ketjen Black (carbon black) and 40 parts of particles made of a crosslinked urethane resin having a number average primary particle diameter of 20  $\mu\text{m}$  were mixed and dispersed to prepare surface layer-forming material 2.

(Preparation Example 3 of Silicone Copolymerization Polyurethane Resin Surface Layer-Forming Material)

Into a reactor fitted with a stirrer, a thermometer, a nitrogen gas-introducing tube and a reflux condenser, charged were 166 parts of  $\epsilon$ -caprolactone, 150 parts of alcohol modified siloxane (exemplified compound 3-6) and 0.04 parts of tetrabutyltitanate, and the system was reacted under nitrogen gas stream at 180° C. for 10 hours to prepare a polysiloxane-polyester copolymer having a number average molecular weight of 4010, an acidic value of 0.35 and a hydroxyl value of 28.

In a mixed solvent of 200 parts of methylethyl ketone and 100 parts of dimethylformamide, dissolved were 150 parts of the above-described copolymer and 27 parts of 1,4-butanediol, and then a solution obtained by dissolving 88 parts of water-added MDI in 192 parts of dimethylformamide was gradually dripped while stirring at 60° C. After dripping was completed, the resulting was reacted at 80° C. for 6 hours to prepare a silicone copolymerization polyurethane resin solution of the present invention. This solution had a viscosity of 31.2 Pa·s (25° C.) at a solid content of 35%.

Further, 100 parts of the resulting silicone copolymerization polyurethane resin, 30 parts of Ketjen Black (carbon black) and 40 parts of particles made of a crosslinked urethane resin having a number average primary particle diameter of 20  $\mu\text{m}$  were mixed and dispersed to prepare surface layer-forming material 3.

(Preparation Example 4 of Silicone Copolymerization Polyurethane Resin Surface Layer-Forming Material)

In a mixed solvent of 200 parts of methylethyl ketone and 150 parts of dimethylformamide, dissolved were 75 parts of a copolymer of foregoing preparation example 3, 75 parts of polyethylene adipate having a number average molecular weight of 2000, an acidic value of 0.28 and a hydroxyl value of 56.0, and 27 parts of 1,4-butanediol, and then a solution obtained by dissolving 93 parts of MDI in 151 parts of dimethylformamide was gradually dripped while stirring at 60° C. After dripping was completed, the resulting was reacted at 80° C. for 6 hours to prepare a silicone copolymerization polyurethane resin solution of the present invention. This solution exhibited high transparency, accompanied with a

viscosity of 40.5 Pa·s (25° C.) at a solid content of 35%. Further, 100 parts of the resulting silicone copolymerization polyurethane resin, 30 parts of Ketjen Black (carbon black) and 40 parts of particles made of a crosslinked urethane resin having a number average primary particle diameter of 20  $\mu\text{m}$  were mixed and dispersed to prepare surface layer-forming material 4.

{Preparation Example 1 of Developing Roller (Example 1)}

After a core metal made of SUS303 (a diameter of 10 mm) as shaft 2 was set to the inside of a roller, the foregoing elastic (base rubber) layer-forming material 1 was injected into a gap portion between the foregoing shaft and the inner circumferential surface of the roller (refer to FIG. 2), and vulcanized while heating at 180° C. for one hour. Subsequently, formwork removal was conducted, and the secondary vulcanizing treatment was further carried out at 200° C. for 4 hours to form elastic layer 3 having a thickness of 5 mm on the outer circumferential surface of shaft 2.

After the shaft with the resulting base rubber layer was removed from the above-described die, and intermediate layer-forming material 1 was formed 15  $\mu\text{m}$  thick on the outer circumferential surface of the base rubber layer, a heat treatment was conducted at 100° C. for one hour to form a layer made of a polyurethane resin-silica hybrid. Further, surface layer-forming material 1 was coated 15  $\mu\text{m}$  thick, a heat treatment was conducted at 100° C. for one hour to form a surface layer made of a silicone copolymerization polyurethane resin, and to obtain a developing roller of the present invention. This roller is designated as developing roller 1.

{Preparation Example 2 of Developing Roller (Example 2)}

A developing roller of the present invention was prepared similarly to preparation example 1 of developing roller, except that intermediate layer-forming material 1 was replaced by intermediate layer-forming material 2 with a thickness of 10  $\mu\text{m}$ , and surface layer-forming material 1 was also replaced by surface layer-forming material 2. This roller is designated as developing roller 2.

{Preparation Example 3 of Developing Roller (Example 3)}

A developing roller of the present invention was prepared similarly to preparation example 1 of developing roller, except that intermediate layer-forming material 1 was replaced by intermediate layer-forming material 3 with a thickness of 12  $\mu\text{m}$ , and surface layer-forming material 1 was also replaced by surface layer-forming material 3. This roller is designated as developing roller 3.

{Preparation Example 4 of Developing Roller (Example 4)}

A developing roller of the present invention was prepared similarly to preparation example 1 of developing roller, except that intermediate layer-forming material 1 was replaced by intermediate layer-forming material 4, and surface layer-forming material 1 was also replaced by surface layer-forming material 4. This roller is designated as developing roller 4.

(Preparation of Surface Layer-Forming Material 1 for Comparative Example)

One hundred parts of an urethane resin (Nipporan 5199, produced by Nippon Polyurethane Industry Co., Ltd.), 30 parts of Ketjen Black, 400 parts of MEK (methylethyl ketone), and 40 parts of particles having a number average primary particle diameter of 20  $\mu\text{m}$ , which are made of a crosslinked urethane resin were mixed and dispersed to prepare surface layer-forming material 1 for a comparative example.

## {Preparation Example 1 of Comparative Developing Roller (Comparative Example 1)}

A comparative developing roller was prepared similarly to preparation example 1 of developing roller, except that intermediate layer-forming material 1 was replaced by bis(1,2-triethoxysilyl)ethane to be evenly coated, and a heat treatment was conducted at 100° C. for one hour. This roller is designated as comparative developing roller 1.

## {Preparation Example 2 of Comparative Developing Roller (Comparative Example 2)}

A comparative developing roller was prepared similarly to preparation example 1 of developing roller, except that surface layer-forming material 1 was replaced by a surface layer-forming material 1 for comparative example. This roller is designated as comparative developing roller 2.

## [Preparation Example of Toner]

## (Preparation Example 1 of Resin Particles)

In a flask fitted with a stirrer, 72.0 g of wax pentaerythritol (tristearic acid ester) was added into a monomer mixture composed of 115.1 g of Styrene, 42.0 g of n-butylacrylate and 10.9 g of methacrylic acid, and dissolved while heating at 80° C. to prepare a monomer solution.

On the other hand, a surfactant solution (aqueous medium) in which 7.0 g of anionic surfactant (sodium dodecylbenzenesulfonate: SDS) was dissolved in 2760 g of ion-exchange water was charged into a separable flask fitted with a stirrer, a thermometer, a cooling tube and a nitrogen gas-introducing tube, and the inner temperature was increased to 80° C. under nitrogen gas stream while stirring at a stirring rate of 230 rpm. Next, the foregoing monomer solution (at 80° C.) was mixed and dispersed in the foregoing surfactant solution (at 80° C.), employing a mechanical homogenizer (CLEARMIX, produced by M Technique Co., Ltd.) with a circulating path to prepare an emulsified liquid in which emulsification particles (oil droplets) having an even particle diameter were dispersed.

An initiator solution in which 0.84 g of polymerization initiator (potassium persulfate: KPS) was dissolved in 200 g of ion-exchange water was added into this dispersion, and this system was heated at 80° C. for 3 hours while stirring to conduct polymerization reaction. A solution in which 7.73 g of polymerization initiator (KPS) was dissolved in 240 g of ion-exchange water was added into the resulting reaction solution, and a mixture composed of 383.6 g of styrene, 140.0 g of n-butylacrylate, 36.4 g of methacrylic acid and 12 g of n-octylmercaptan was dripped spending 100 minutes, after the temperature was increased to 80° C. spending 15 minutes. After stirring this system at 80° C. for 60 minutes, a resin particle dispersion containing wax {hereinafter, referred to as "Latex (1)"} was prepared by cooling this system to 40° C.

## (Preparation Example 1 of Colorant Dispersion)

On the other hand, 9.2 g of n-dodecyl sodium sulfate was dissolved in 160 g of ion-exchange water while stirring. Twenty gram of carbon black (Mogul L, produced by Cabot Corporation) as a colorant was gradually added while stirring this solution, and the system was subsequently dispersed employing a mechanical homogenizer (CLEARMIX, produced by M Technique Co., Ltd.) to prepare a colorant particle dispersion {hereinafter, referred to as "colorant dispersion (1)"}.

A particle diameter of the colorant particle in colorant dispersion (1), which was measured employing an electrophoresis light-scattering photometer (ELS-800, manufactured by Ohtsuka Denshi Co., Ltd.), was 120 nm in weight average particle diameter.

## (Preparation Example 2 of Colorant Dispersion)

A colorant particle dispersion {hereinafter, referred to as "colorant dispersion (2)"} was prepared similarly to preparation example 1 of colorant dispersion, except that 20 g of carbon black was replaced by 20 g of a pigment "C.I. pigment yellow 74". A particle diameter of the colorant particle in the resulting colorant dispersion (2), which was measured employing an electrophoresis light-scattering photometer (ELS-800, manufactured by Ohtsuka Denshi Co., Ltd.), was 120 nm in weight average particle diameter.

## (Preparation Example 3 of Colorant Dispersion)

A colorant particle dispersion {hereinafter, referred to as "colorant dispersion (3)"} was prepared similarly to preparation example 1 of colorant dispersion, except that 20 g of carbon black was replaced by 20 g of a quinacridone based magenta pigment "C.I. pigment red 122". A particle diameter of the colorant particle in the resulting colorant dispersion (3), which was measured employing an electrophoresis light-scattering photometer (ELS-800, manufactured by Ohtsuka Denshi Co., Ltd.), was 120 nm in weight average particle diameter.

## (Preparation Example 4 of Colorant Dispersion)

A colorant particle dispersion {hereinafter, referred to as "colorant dispersion (4)"} was prepared similarly to preparation example 1 of colorant dispersion, except that 20 g of carbon black was replaced by 20 g of a phthalocyanine based cyan pigment "C.I. pigment blue 15:3". A particle diameter of the colorant particle in the resulting colorant dispersion (4), which was measured employing an electrophoresis light-scattering photometer (ELS-800, manufactured by Ohtsuka Denshi Co., Ltd.), was 120 nm in weight average particle diameter.

## (Preparation Example K1 of Colorant Particle)

Into a reaction vessel (four-necked flask) fitted with a thermometer, a cooling tube, a stirrer with two stirring blades having a crossing angle of 20°, and a shape-monitoring device, charged were 1250 g (solid content conversion) of latex (1), 2000 g ion-exchange water and the total amount of colorant dispersion (1), the inner temperature was adjusted to 25° C., and an aqueous 5 mol/liter sodium hydroxide solution was subsequently added into this dispersion mixture solution to adjust pH to 10.0. Next, an aqueous solution in which 52.6 g of magnesium chloride-hexahydrate was dissolved in 72 g of ion-exchange water was added at 25° C. for 10 minutes while stirring. After this, the temperature of this system was immediately increased to 95° C. at a temperature increasing rate of 14° C./min, spending 5 minutes.

In this situation, the particle diameter of associated particles was measured employing "Multisizer 3, manufactured by Beckman Coulter Co., Ltd.", and when the volume-based median diameter reached 6.5 µm, particle growth was terminated by adding an aqueous solution in which 115 g of sodium chloride was dissolved in 700 g of ion-exchange water. Furthermore continuing a fusing treatment and then conducting a ripening treatment while stirring at a stirring rotation speed of 120 rpm at a liquid temperature of 90° C. for 8 hours, this system was cooled to 30° C. at a temperature cooling rate of 10° C./min, pH was adjusted to 3.0 by adding a hydrochloric acid, and then stirring was terminated.

The resulting particles were filtrated, and repeatedly washed with ion-exchange water to conduct a submerged classification treatment employing a centrifugal separator. After this, prepared was the colorant particle {hereinafter, referred to as "colorant particle (K1)"} having a moisture content of 1.0% obtained via a drying process employing a flash jet dryer.

## 31

## (Preparation Example Y1 of Colorant Particle)

Colorant particle (Y1) was prepared similarly to preparation example K1 of colorant particle, except that the total amount of colorant dispersion (1) was replaced by the total amount of colorant dispersion (2).

## (Preparation Example M1 of Colorant Particle)

Colorant particle (M1) was prepared similarly to preparation example K1 of colorant particle, except that the total amount of colorant dispersion (1) was replaced by the total amount of colorant dispersion (3).

## (Preparation Example C1 of Colorant Particle)

Colorant particle (C1) was prepared similarly to preparation example K1 of colorant particle, except that the total amount of colorant dispersion (1) was replaced by the total amount of colorant dispersion (4).

## (Preparation of Toner)

Into the above-described colorant particles, added were 0.8 parts by weight of hydrophobic silica having a number average primary particle diameter of 12 nm and a hydrophobic degree of 65, and 0.5 parts by weight of hydrophobic titania having a number average primary particle diameter of 30 nm and a hydrophobic degree of 55, and the resulting was mixed employing a Henschel mixer to prepare each toner. These are designated as black toner 1, yellow toner 1, magenta toner 1 and cyan toner 1, respectively.

## [performance Evaluation]

## (Interlayer Adhesion)

As shown in FIG. 3(a), incisions with a width of 2.5 cm indicated by dashed line X were made along with outer circumferential surface of surface layer 5 at the roller center portion, and an incision (dashed line Y) was further made in the shaft direction on surface layer 5. Surface layer 5 was slightly peeled from the incised portion, and then the end of peeled surface layer 5 was raised vertically employing "Auto-graph AGS, manufactured by Shimadzu Corporation" (Z-pointing arrow direction), as shown in FIG. 3(b). How much force was necessary to start peeling off the surface layer

## 32

The resin layer was raised specifically at a speed of 100 mm/min. In the process of increasing a load value to 20 N, a load value in which the resin layer was possible to be raised with no increase of load was determined.

5 The evaluation was made according to the following criteria employing this value.

A: A load value to start peeling off is at least 10.0 N.

B: A load value to start peeling off is at least 4.0 N and less than 10.0 N.

10 C: A load value to start peeling off is less than 4.0 N.

## (Image Evaluation)

15 Three thousand A4 size practical prints were evaluated in a pixel ratio of 20% (5% of each color of yellow, magenta, cyan and black in full color mode) by utilizing the resulting developing roller installed in a color laser printer (Magicolor 2300DL, manufactured by Konica Minolta Business Technologies, Inc.). Fine line reproduction (resolution), density unevenness and fog density were evaluated at room-temperature and low-humidity (20° C. and 10% RH) at the initial 20 stage and after printing 3000 prints.

## Fine Line Reproduction (Resolution)

Fine line portions were enlarged at a factor of 10, employing a loupe to evaluate fine line reproduction (resolution, lines per mm).

## 25 Density Unevenness

30 A4 size solid image (a pixel ratio of 100%) was printed at the initial stage and after printing 3000 prints. The reflection density at each of 10 portions selected at random on the printed A4 size solid image (a pixel ratio of 100%) was measured employing a Macbeth reflection densitometer RD-918 to evaluate the density unevenness from the difference between maximum and minimum values of solid image density.

## 35 Fog

In order to evaluate fog density, the white portion was measured employing a Macbeth reflection densitometer RD-918, and the fog density was evaluated via relative reflection density in which reflection density of a paper sheet was set to "0".

TABLE 1

| No.                   | Developing roller No.           | Interlayer adhesion | Image evaluation |                    |       |                            |                    |       |
|-----------------------|---------------------------------|---------------------|------------------|--------------------|-------|----------------------------|--------------------|-------|
|                       |                                 |                     | At initial stage |                    |       | After printing 3000 prints |                    |       |
|                       |                                 |                     | *1               | Density Unevenness | Fog   | *1                         | Density Unevenness | Fog   |
| Example 1             | Developing roller 1             | A                   | 6                | 0.01               | 0.001 | 6                          | 0.01               | 0.001 |
| Example 2             | Developing roller 2             | A                   | 6                | 0.01               | 0.000 | 6                          | 0.01               | 0.001 |
| Example 3             | Developing roller 3             | A                   | 6                | 0.01               | 0.001 | 6                          | 0.01               | 0.002 |
| Example 4             | Developing roller 4             | A                   | 6                | 0.01               | 0.000 | 6                          | 0.01               | 0.001 |
| Comparative example 1 | Comparative developing roller 1 | C                   | 6                | 0.01               | 0.001 | 4                          | 0.15               | 0.012 |
| Comparative example 2 | Comparative developing roller 2 | C                   | 6                | 0.01               | 0.001 | 4                          | 0.18               | 0.015 |

\*1: Fine line reproduction (resolution)

out of an adjacent layer under the surface layer was measured to evaluate the interlayer adhesion.

65 As is clear from Table 1, it is to be understood that Examples 1-4 of the present invention exhibit excellent interlayer adhesion between resin layers composed of two layers,

## 33

and toner additive adhesion that possibly causes image blur and fog can be prevented by a surface layer having low surface energy, whereby excellent images can be obtained even after printing 3000 prints.

On the contrary, Comparative examples 1 and 2 of the present invention exhibit inferior image blur and fog properties possibly caused by peeling of a surface layer because of insufficient adhesion between resin layers, and by foreign matters adhered to the surface layer.

## Effect of the Invention

The present invention is possible to provide a developing roller in which increase of residual potential is inhibited during repetitive operation without deteriorating interlayer adhesion, and prepared is a layer immediately below the surface capable of preventing fog caused by toner scattering, accompanied with a surface layer capable of preventing stains formed from foreign matters adhered to the surface, as well as preventing image unevenness since toner electrification is even under the presence of appropriate elasticity, and also to provide a image forming method employing the developing roller.

What is claimed is:

1. A developing roller comprising an elastic layer made of silicone rubber provided around a conductive shaft, and a plurality of resin layers further provided on the elastic layer, wherein a surface layer among the resin layers comprises silicone copolymerization polyurethane as a principal component; and

## 34

a layer immediately below the surface layer comprises a polyurethane resin-silica hybrid as a principal component.

2. The developing roller of claim 1, wherein a silane moiety content in the polyurethane resin-silica hybrid is 1.0-30.0% by weight.

3. The developing roller of claim 1, wherein the polyurethane resin-silica hybrid comprises a urea bond.

4. An image forming method comprising the steps of:

(a) conveying a developer comprising a toner to a developing region with a developing roller; and

(b) developing an electrostatic latent image formed on an electrostatic latent image carrier for visualization, wherein the developing roller comprises an elastic layer made of silicone rubber provided around a conductive shaft, and a plurality of resin layers further provided on the elastic layer; and

wherein a surface layer among the resin layers comprises silicone copolymerization polyurethane as a principal component, and a layer immediately below the surface layer comprises a polyurethane resin-silica hybrid as a principal component.

5. The image forming method of claim 4, wherein a silane moiety content in the polyurethane resin-silica hybrid is 1.0-30.0% by weight.

6. The image forming method of claim 4, wherein the polyurethane resin-silica hybrid comprises a urea bond.

\* \* \* \* \*